

## UNITED STATES PATENT OFFICE

2,182,612

PRODUCT FOR USE AS NONRUSTING AND  
NONCORRODING ANTIFREEZING MIX-  
TURESCyrus D. Eaton, Lansdowne, Pa., assignor to The  
American Distilling Company, Incorporated,  
Philadelphia, Pa.No Drawing. Application January 30, 1937,  
Serial No. 123,144

2 Claims. (Cl. 252—5)

This invention relates to a product and an improved process for preventing corrosion of cooling systems of internal combustion engines and, in particular, is directed to an improvement of 5 the corrosion preventive property of freezing point depressants to be used with cooling liquids of said cooling systems, and more particularly to the attainment of that effect by the use of sodium salicylate.

10 An object of the invention is to provide a composition which, when added to the usual cooling liquid used in internal combustion engines, will prevent the rusting and corrosion of the ferrous, as well as the various nonferrous metals of such 15 cooling systems.

Another object of the invention is to provide a composition of high efficiency as a cooling liquid for use in internal combustion engines.

Another object of the invention is to provide 20 a composition of high efficiency as a freezing point depressant of the cooling liquid used in internal combustion engines.

Another object of the invention is to provide 25 a composition which will readily mix with and continue mixed with the usual cooling liquid used in internal combustion engines.

Another object of the invention is to furnish 30 an improved alcoholic antifreeze mixture, containing therein small quantities of ingredients which do not deleteriously effect the alcohol and which minimize or suppress the corrosion of the metals of the cooling system upon dilution of the alcohol when used in the cooling system.

Among the various substances used by 35 automobile owners to prevent freezing of the liquid cooling media of the engines, alcohol has played a prominent part. The freezing point of absolute ethyl alcohol is about minus (—) 112° C. Alcohol depresses the freezing point of water and 40 such depression depends upon the concentration of the alcohol in the water. The greater the concentration of alcohol, the lower is the freezing point of the mixture.

Automobile owners, knowing the volume of the 45 cooling systems of their engines, guard against expected minimum temperatures by adding appropriately measured quantities of alcohol. Charts are readily available for the automobile owners, which stipulate the quantities of alcohol to be added to the cooling systems of various 50 makes of automobiles for various operating temperatures.

Alcohol by itself has, however, not proved entirely satisfactory as an antifreeze. This has 55 been due to the fact that the metals of the sys-

tems, in which the cooling liquids containing the alcohol circulate, undergo rusting and corrosion.

The damage caused by such rusting and corrosion is considerable. On the one hand there results actual deterioration of the metals and parts attacked. Radiators begin to leak; solder is eaten away; the joints disintegrate; and the cooling system fails to hold the liquid. Furthermore, the products resulting from the corrosion are distributed by the cooling liquid through the system. The solid products especially tend to clog the radiators and the other parts of the cooling system. As a result of the clogging, the circulation of the cooling liquid is materially interfered with, causing overheating of the engine, boiling out of the liquid, and damage to the engine. The boiling of the liquid also results in loss of the antifreeze composition.

Ferrous, as well as nonferrous metals, are employed in the construction of the above described cooling systems. The metals are sometimes joined and connected to each other by means of solder. Effective and inexpensive compositions of alcoholic antifreezes, which will act as rust 20 and corrosion preventives of both types of metals and alloys of the nonferrous metals, have been sought.

Among these compositions use has been made 30 of light hydro-carbon mineral oils, such as kerosene, dispersed in absolute or high-proof alcohol. The light hydro-carbon mineral oils have been known to function as rust and corrosion preventives. Such compositions, however, are not always stable on dilution and the oils separate 35 out, with consequent loss of the corrosion preventive effect of the light hydro-carbon mineral oils. The separation of the light hydro-carbon mineral oil from the alcohol on dilution is suppressed by the addition to the mixture of a small 40 quantity of sulfonated castor oil. Such a mixture is an effective rust and corrosion preventive, when used for antifreezing purposes.

I have found that, although compositions of 45 alcohol, light hydrocarbon mineral oil, such as kerosene, and a small quantity of sulfonated castor oil are rust and corrosion preventives, they sometimes do stain the metallic surfaces, with subsequent discoloration of the liquid medium. This staining and discoloration may, however, be 50 obviated, as I have found, by the addition to such a composition of a small quantity of sodium salicylate.

When a composition, which consists simply of 55 completely denatured alcohol and sodium sali-

cylate in the proportions of one-tenth of a gram of the salicylate to 100 cubic centimeters of the alcohol, is used for test purposes, I have found that it will produce rusting within twenty-four hours. If, however, there be added to the same composition one cubic centimeter of kerosene and three one-hundredths of a cubic centimeter of sulfonated castor oil, a test solution so made results in complete inhibition of stain formation on the metallic surface for a period of nine days and the liquid remains undiscolored.

I have found that the sulfonated castor oil content in a composition of the foregoing character may range in the proportions of one one-hundredth of a cubic centimeter to one-tenth of a cubic centimeter for each cubic centimeter of the light hydrocarbon mineral oil. An effective specific composition consists of one hundred cubic centimeters of completely denatured alcohol, four and two-tenths cubic centimeters of kerosene, three-tenths of a cubic centimeter of sulfonated castor oil and one-tenth to four-tenths of a gram of sodium salicylate.

A composition of the foregoing character may be used for testing its staining effect and non-discolorable property as follows:

One volume of the foregoing composition is diluted with three volumes of tap water. There is then immersed into the liquid a bundle of strips of iron, brass, aluminum and solder. The liquid is maintained at a temperature from 170° Fahrenheit to 175° Fahrenheit. Water is added from time to time to compensate for evaporative loss.

A test such as the foregoing demonstrates effectively the non-staining character of the composition. It will also be observed that the liquid remains undiscolored.

It is to be understood that the proportions given in the foregoing example are merely illustrative.

It is also to be understood that either anhydrous alcohol, or high-proof alcohol, may be used for the completely denatured ingredient.

The composition, which has just been described, is highly effective as a rust and corrosion preventive, even when it is diluted for use as an antifreeze. The quantity to be used as an antifreeze may be computed according to the volume of the cooling system and the temperatures in which the engine is expected to operate. This composition is easily prepared, is cheap, and unusually stable during long periods of storage. It disperses rapidly and completely throughout the cooling liquid.

Having thus described my invention, I claim:

1. A noncorroding "antifreeze" consisting of

*Approximate proportions*

|                               |                   |                  |    |
|-------------------------------|-------------------|------------------|----|
| Denatured alcohol             | cubic centimeters | 100              | 20 |
| Light hydrocarbon mineral oil | cc                | from 1.0 to 4.2  | 25 |
| Sulfonated castor oil         | cc                | from 0.03 to 0.3 |    |
| Sodium salicylate             | grams             | from 0.1 to 0.4  |    |

2. A noncorroding "antifreeze" consisting of

*Approximate proportions*

|                       |                   |                  |    |
|-----------------------|-------------------|------------------|----|
| Denatured alcohol     | cubic centimeters | 100              | 30 |
| Kerosene              | do                | from 1.0 to 4.2  |    |
| Sulfonated castor oil | do                | from 0.03 to 0.3 |    |
| Sodium salicylate     | grams             | from 0.1 to 0.4  | 35 |

CYRUS D. EATON.